

(No Model.)

E. T. GREENFIELD & J. NAGEL.  
TUBE.

No. 442,090.

Patented Dec. 2, 1890.



Witnesses

Morris S. Clark

*W. F. Clark*

Inventors  
Edwin T. Greenfield  
Johannes Nagel  
By their Attorney

*John Nagel*

BEST AVAILABLE COPY

# UNITED STATES PATENT OFFICE.

EDWIN T. GREENFIELD AND JUNIUS NAGEL, OF NEW YORK, N. Y., ASSIGNEES,  
BY MESNE ASSIGNMENTS, TO THE INTERIOR CONDUIT AND INSULATION  
COMPANY.

## TUBE.

SPECIFICATION forming part of Letters Patent No. 442,090, dated December 2, 1890.

Application filed May 27, 1890. Serial No. 353,362. (No model.)

*To all whom it may concern:*

Be it known that we, EDWIN T. GREENFIELD, a citizen of the United States, and JUNIUS NAGEL, (who has declared his intention of becoming a citizen of the United States,) both residing at New York city, in the county and State of New York, have invented a new and Improved Tube, of which the following is a specification.

The advantages of employing tubes possessing insulating qualities as conduits for electric conductors has long been known. Among other kinds of tubes used have been those formed by highly compressing paper-pulp into the desired form and depending upon the compressed pulp only for insulation. Another and the most common kind for economical tubes has been a tube formed of layers of paper coated with a bituminous compound, as pitch, which served both to retain the tube in proper form and add to its insulating properties. This latter tube was not homogeneous, and proved objectionable in use, as did the first-mentioned kind, notwithstanding any advantages they might possess from a standpoint of economy in first cost, in that among other things they were affected by dampness to such a degree as to materially lessen their durability and insulating properties. It has also been proposed to use tubes of a bituminous compound combined with a material added in a pulp form, the tube being made by squirting the mixture through a die. This form of tube is difficult of manufacture, and therefore expensive, and the tubes produced were likely to be irregular in composition, besides it being impossible to make them of considerable length.

The tube which we have invented is economical in first cost, is homogeneous, possesses high insulating properties, is strong, durable, and not affected by hygrometric or ordinary thermal changes; and it consists, essentially, of a formed base of two or more thickness or layers of a porous fibrous material—such as felt paper—and a filling of a bituminous material or compound—such as black petroleum-pitch—combined with the porous fibrous material throughout its mass, the whole forming a compound tube possessing the characteris-

ties above mentioned and distinguishable from tubing heretofore treated with a bituminous compound by its greater density throughout its mass, which will appear by cutting, which will show that the tube has lost almost wholly the physical structure of its component materials and assumed new characteristics possessed by none of those materials separately. The brittle character of the bituminous material or compound, which would be a serious objection to its use alone for a tube, is supplemented by the fibrous character of the formed base, which imparts the desirable strength, and the hygroscopic character of the formed base is supplemented by the bituminous compound, which effectually obviates all tendency in the compound tube to absorb moisture.

The fibrous porous material which I make use of as a base may be either of a vegetable nature, as sheathing-paper, or of an animal nature, as felt paper, or of a mineral nature, as asbestos. When made of animal or vegetable fiber, the base is first formed in the desired shape, preferably for large sizes, by serving longitudinal layers thereof one over the other, each layer breaking joint with its next inner layer, and for small sizes by a longitudinal core with a spiral wrap or wrappings. When asbestos is used as the base, the tube is first formed in any desirable manner—as, for instance, by wrapping a sheet of what is known as "asbestos paper" in concentric layers on a mandrel. The material which we prefer to use as the base for the tubes of large size is that known as "felt paper," which possesses an exceedingly open porous structure, well adapted for combining throughout its mass with the filling material or compound.

For smaller sizes of tubing we prefer to make use as a base of what is known as "sheathing-paper," which possesses a somewhat less open or porous structure than the felt paper, but is yet sufficiently open to combine with a large quantity of the filling material or compound throughout its mass.

The large size tubing is especially adapted for use as a conduit in a system of underground distribution where difficulties from moisture are most to be apprehended, while

the small tubing is especially adapted for use as a conduit for interior systems of distribution where danger from moisture is less great, and where, therefore, the small sizes do not require the presence of so much compound as do the conduits for underground work. The paper base having been shaped from the required quality of animal or vegetable porous material, then constitutes what I have termed a "formed base," and is ready to have combined with it the filling compound or material, which is done in the following manner: The compound is maintained in a suitable kettle in a liquid condition by heat, the best working condition being attained when the compound is reduced to a state so that it will run freely like water. When in this condition, the heat of the filling material is such that if the paper bases were left in it for any length of time they would become charred, and thereby seriously impaired. To obviate this, we immerse the bases in the filler for a brief period, withdraw them rapidly, and then allow them to remain out of the filler for a period, preferably somewhat longer than the period of immersion. The bases are again immersed and the immersion followed by a second period of rest, and this operation of alternate immersions and rests is continued until there is a thorough combination of the filling material with the material of the bases.

For a base one inch in internal diameter with a wall three-eighths inch thickness made of felt paper we find that the following periods of immersions and rests, using black petroleum-pitch as the filler, will produce a compound tube homogeneous in physical characteristics.

| No. of immersions. | Immersion minutes. | Rests minutes. |
|--------------------|--------------------|----------------|
| 1                  | $\frac{1}{4}$      | 3              |
| 2                  | $\frac{1}{2}$      | $2\frac{1}{2}$ |
| 3                  | $\frac{3}{4}$      | 2              |
| 4                  | 1                  | $1\frac{1}{2}$ |
| 5                  | $1\frac{1}{2}$     | $1\frac{1}{2}$ |
| 6                  | 2                  | $1\frac{1}{2}$ |
| 7                  | $2\frac{1}{2}$     | 1              |
| 8                  | 3                  | 1              |
| 9                  | $3\frac{1}{2}$     | 1              |
| 10                 | 4                  | 1              |
| 11                 | $4\frac{1}{2}$     | 1              |
| 12                 | 5                  | $\frac{3}{4}$  |
| 13                 | 5                  | $\frac{1}{2}$  |
| 14                 | 5                  | $\frac{1}{2}$  |
| 15                 | 5                  | —              |

55 A twelve-inch length of felt base of the diameter and thickness of wall above stated will weigh four ounces. When combined with the filler by the process above set out, it will weigh twelve ounces without having increased perceptibly in dimensions. Such a compound tube is well adapted for underground conduits.

For a base of sheathing-paper of three-eighths inch internal diameter with a wall one-sixteenth inch thickness, using black petroleum-pitch as a filler, we find that the follow-

ing periods of rests and immersions will produce a homogeneous tube.

| No. of immersions. | Immersion minutes. | Rests minutes. | 70 |
|--------------------|--------------------|----------------|----|
| 1                  | $\frac{1}{4}$      | $1\frac{1}{2}$ |    |
| 2                  | $\frac{1}{2}$      | $1\frac{1}{2}$ |    |
| 3                  | $\frac{3}{4}$      | 1              |    |
| 4                  | 1                  | $\frac{3}{4}$  |    |
| 5                  | $1\frac{1}{4}$     | $\frac{1}{2}$  | 75 |
| 6                  | $1\frac{1}{2}$     | —              |    |

80 A twelve-inch length of a base made of sheathing-paper having an internal diameter of three-eighths inch and a wall of one-sixteenth of an inch in thickness will weigh one and three-quarter ounces. When combined with the filler by the process above set forth it will weigh two and three-quarter ounces without having increased perceptibly in dimensions. Such a tube is well adapted as a conduit for interior wiring.

85 When a mineral fibrous material is used as a base, the same may have the filler combined with it without employing the process of alternate immersions and rests above set forth, as there is no danger of charring the mineral fiber, although even with mineral fiber we prefer to employ this process for combining the base and filler.

90 We have described the new tube of our invention as especially useful as a conduit for electric conductors; but it is apparent that it may be applied to many other uses—as, for instance, for the conveyance of fluids and 100 gases, and for speaking-tubes, &c.

95 In the accompanying drawings, forming a part of this specification, Figure 1 is a plan view of the formed base for a large-sized tube. Fig. 2 is a transverse section thereof. Fig. 3 105 is a plan view of the formed base for a tube of small size. Fig. 4 is a transverse section thereto. Fig. 5 is an end view of a formed base of asbestos, and Fig. 6 is a cross-section of any of the above tubes after the filler has 110 been combined therewith.

115 In Figs. 1 and 2, *a* is the inner longitudinally-served layer of felt paper, or other suitable porous fibrous material. Preferably this layer is arranged so that its meeting edges *b* abut to form the seam *b*. *c* is the next longitudinally-applied layer, the edges of which also abut, and are arranged so that the seam *d* breaks joint with the seam *b*. *e* is the outer layer, applied in the same manner as the layers *a* and *c*, and the seam *f* breaks joint with the seam *d* of the next inner layer. A strip of thin paper *g* may be pasted over the seam *f*, so that the formed base will be held in its true shape while being combined with the filler. As many layers of the felt or other suitable material may be employed as may be found desirable to make the necessary thickness of tube, depending, of course, upon the thickness of each individual layer.

130 In Figs. 3 and 4, *h* is the internal core of the formed base, which is a fillet of sheathing-paper or other suitable material having a seam *i*. Around this longitudinal seamed

core a spiral wrap or wrappings of suitable material *j* are applied. This sheathing of paper is not quite so open or porous as is the felt paper; but it is sufficiently open and 5 porous to combine with a considerable quantity of the filling material or compound.

Fig. 5 shows a sheet of mineral fiber asbestos formed by a single sheet wrapped in concentric layers.

10 Fig. 6 is a cross-section of a treated tube, showing, as far as a drawing can, that when the filler is combined with the formed base the result is a tube homogeneous throughout its mass.

15 What we claim as our invention is—

1. As a new article of manufacture, a compound tube comprising a formed base of two or more thicknesses of a porous fibrous ma-

terial and a filling of bituminous material or compound combined with said formed base *so* throughout its mass, substantially as specified.

2. As a new article of manufacture, a compound tube having a formed base of two or more thicknesses of paper and a filling of a *25* bituminous compound combined with said base throughout its mass, substantially as specified.

This specification signed and witnessed this 15th day of May, 1890.

EDWIN T. GREENFIELD  
JUNIUS NAGEL.

Witnesses:

C. S. CHAMPION,  
W. PELZER.